

## UNITED STATES PATENT OFFICE

SAMUEL WHYTE, OF REDHILL, ENGLAND, ASSIGNOR TO VICTOR TALKING MACHINE COMPANY, A CORPORATION OF NEW JERSEY

## SOUND RECORD

No Drawing. Application filed January 28, 1931, Serial No. 511,927, and in Great Britain February 5, 1930.

The present invention relates to laminated disc sound records, each layer of which comprises a cellulose derivative and a plastifier.

It has been proposed, in connection with records consisting of three layers, all containing a cellulose ester, to provide the internal layer with a larger content of plasticising material than the external layers contain and thus obtain a record, the internal layer of which has a different coefficient of expansion to that of the external layers.

In the record of the present invention, all the layers of which comprise a cellulose derivative and a plastifier, the external or surface layers contain filling material and in an amount in excess of any contained in the internal layer and in addition have a lower plastifier content than the latter, the internal layer being thus made softer and more flexible than the external or surface layers. By filling material is meant any inert material such as barytes, slate powder, silica, black oxide of iron or the like.

The present invention provides a record of a limp nature which tends to lie flat under all conditions, since the internal layer has not the resilient qualities of the outside layers. A further advantage of the record of the present invention is that pressing is facilitated since the hard material necessary for the surface will flow more easily in pressing with the softer core below and it is thus easier to obtain a perfect surface free from air marks.

The content of plastifier used in the core or internal layer of a record according to the invention may vary from one-half to one-and-a-half times that of cellulose derivative present in the core or internal layer, while the content of filling material in this layer preferably should not constitute more than 25% by weight of the total core material.

Examples of compositions preferred for the surface layers of a record according to the present invention are as follows:

|                            | Per cent<br>by weight |
|----------------------------|-----------------------|
| (1) (1) Slate powder       | 32.5                  |
| Plastifier (amyl tartrate) | 18.5                  |
| Cellulose acetate          | 46.0                  |
| Pigment                    | 3.0                   |
| (2) Barytes                | 45.0                  |
| Plastifier                 | 14.8                  |

|     |                            |      |
|-----|----------------------------|------|
|     | Cellulose acetate          | 37.2 |
|     | Pigment                    | 3.0  |
| (3) | Silica                     | 29.2 |
|     | Black oxide of iron        | 14.6 |
|     | Plastifier                 | 18.0 |
|     | Cellulose acetate          | 36.0 |
|     | Carbon black               | 1.1  |
|     | Nigrosine                  | 1.1  |
| (4) | Black oxide of iron        | 58.3 |
|     | Carbon black               | .85  |
|     | Nigrosine                  | .85  |
|     | Plastifier (amyl tartrate) | 20.0 |
|     | Cellulose acetate          | 20.0 |

Examples of compositions preferred for the internal layer are as follows, the proportions in this case also being by weight:

|                   | 1        | 2        | 3        |
|-------------------|----------|----------|----------|
|                   | Per cent | Per cent | Per cent |
| Cellulose acetate | 66       | 53       | 31.6     |
| Plastifier        | 33       | 35       | 47.4     |
| Pigment           | 1        | 2        | 1.0      |
| Filler            | 10       | 20       | 20.0     |

It is also found advantageous sometimes to incorporate a small quantity of resin, for example 4 to 5% by weight, in the core material, especially when the latter contains filling material.

The layers of a record according to the present invention may be prepared by any suitable method. For example, in one method the components are mixed together with two to three times their total weight of a solvent consisting of, for example, 75% acetone, 10% methylated spirits and 15% methyl ethyl ketone, to form a paint which is spread on to a canvas belt and dried thereon. The film formed is then stripped from the belt, seasoned and blanked out into discs of suitable size.

In an alternative method, the components are formed into a plastic mass by malaxation with a volatile solvent, such as acetone, on heated rolls at a temperature preferably below the boiling point of the solvent and then squeezed between heavy rollers to form sheets of the desired thickness. These sheets are seasoned and blanked out into discs of suitable size.

The various layers are united under heat and pressure to form a record preferably at the same moment as the sound trace is imparted thereto. The preferred form of rec-

ord consists of a softer layer having a hard layer attached to each side thereof. In a flexible record of this type, the core may be .010" thick and each external layer .005" 5 thick, the complete record being approximately .02" thick.

Although I have shown and described certain specific embodiments of my invention, I am fully aware that many modifications 10 thereof are possible. My invention, therefore, is not to be restricted except insofar as is necessitated by the prior art and by the spirit of the appended claims.

I claim as my invention:

- 15 1. A laminated disc sound record comprising a plurality of layers of a cellulose derivative and a plastifier wherein the quantity of plastifier present in the internal layer is not less than one half that of the cellulose derivative present in said layers.
- 20 2. A laminated disc sound record comprising a plurality of layers of a cellulose derivative and a plastifier, the internal layer containing filling material in an amount not more than 25% by weight of the material forming said layer and having a greater plastifier content than said inner layers, said other layer being softer and more flexible than said other layer.
- 25 3. A laminated disc sound record comprising

ing a plurality of layers of a cellulose derivative and a plastifier wherein the quantity of plastifier present in the internal layer does not exceed one and a half times that of cellulose derivative present in said layers, 70 said internal layer also containing a filling material in an amount not more than 25% by weight of the material forming said layer.

4. A laminated disc sound record comprising a plurality of layers of a cellulose derivative and a plastifier wherein the quantity of plastifier present in the internal layer is not less than one half that of the cellulose derivative present in said layers, said internal layer also containing a filling material in an amount not more than 25% by weight of the material forming said layer. 75

5. A laminated disc sound record comprising a plurality of layers of a cellulose derivative and a plastifier wherein the quantity of plastifier present in the internal layer is not less than one half that of cellulose derivative present nor in excess of one and one half times that of cellulose derivative present in said layer, said internal layer also containing a filling material in an amount not more than 25% by weight of the material forming said layer. 80 85

SAMUEL WHYTE.

95

35

100

40

105

45

110

50

115

55

120

60

125

65

130